

Feb. 24, 1931.

A. L. FEILD

1,794,068

PROCESS OF MAKING OPEN HEARTH STEEL

Filed July 29, 1926



Inventor

Alexander L. Feild

By Barnes, Townsend & McKinney

Attorneys.

## UNITED STATES PATENT OFFICE

ALEXANDER L. FEILD, OF CANTON, OHIO, ASSIGNOR, BY MESNE ASSIGNMENTS, TO REPUBLIC STEEL CORPORATION, OF YOUNGSTOWN, OHIO, A CORPORATION OF NEW JERSEY

## PROCESS OF MAKING OPEN-HEARTH STEEL

Application filed July 29, 1926. Serial No. 125,794.

The present invention comprises a procedure for the manufacture of steel by the open hearth process. In accordance with this invention, the removal of carbon during refining is caused to take place at that rate which is most advantageous from the standpoints (1) of obtaining a product characterized by maximum cleanliness and freedom from non-metallic inclusions (usually oxides 5 and silicates of iron or manganese), or (2) of obtaining a product of the highest degree of cleanliness possible with any selected rate of furnace production. The novel features 10 of the process have to do with methods for determining what is the slag composition corresponding to the particular advantage or combination of advantages sought, for modifying the slag so that it displays this advantageous composition and for maintaining 15 the desired composition while the refining reactions are in progress.

In what follows, discussion is directed in particular to steel-making in the basic-lined open hearth furnace. However, the invention 20 is not considered to be restricted to the basic process.

It has hitherto been common practice in basic open hearth "melting" to proceed more or less in accordance with a certain standardized program, subject however to considerable flexibility, even in the case of a fixed charge composition. This procedure in its 30 detailed aspects is familiar to those skilled in the art and need not be described here. Attention is directed, however, to the fact that the process is complex and that it is characterized by wide variability even when conducted by melters of acknowledged skill 35 and experience in the art, and in furnaces of modern design. For instance, in the case of thirty-eight 100-ton heats of plain carbon steel designated for a product whose carbon content was fixed by specification between the limits of 0.06-0.12% and made by ordinary practice in a single furnace from a 40 charge mixture containing 45% pig iron and 55% steel scrap of reasonably uniform grade and analysis, the amount of ore used varied from 0 to 9000 lbs., the melting time from 45 7 hrs. 15 mins. to 12 hrs. 20 mins., and the fin-

ishing time from 35 mins. to 4 hrs. 40 mins. The carbon content of the metal bath at melting varied from 1.40% to about 0.25%, and the carbon content of the finished steel from 0.06 to 0.11%. 55

During the progress of a heat, the melter has for guidance in timing the iron oxide or ore additions and in deciding upon the weight of each ore addition, the following factors: (1) the intangible factor termed 60 "personal experience", (2) the carbon content of the metal bath at arbitrarily determined intervals, (3) in visually estimated (or measured) temperature of the slag, (4) the temperature of the metal beneath the slag 65 as estimated by any one of a number of approximate methods, all of which involve a large element of judgment, (5) the rate of carbon oxidation at any selected time, as estimated from the vigor and extent of evolution 70 or bubbling of gas (CO and CO<sub>2</sub>) through the slag. When necessary, analysis of the metal bath for manganese, phosphorus, sulphur, and other elements is made to determine whether or not the steel will meet specifications. 75 The presence of an excess of iron oxide in the slag at the end of the refining stage is a fruitful source of the objectionable non-metallic inclusions, above referred to, and this objection can be obviated by my method. 80

I have discovered that the open hearth process may be more carefully controlled and uniformity in product insured by a proper adjustment of the iron oxide content of the slag during the various stages of the finishing or refining period. This adjustment cannot be made until the initial iron oxide content of the slag at melting is determined by chemical analysis or by other suitable method. If this iron oxide content is lower 85 than the value which has been determined to be advantageous by means of the novel method to be described below, a sufficient amount of iron ore or other oxide of iron is added to bring the iron oxide content up to the desired value. If desired, the ore may be added in successive small additions. If the initial iron oxide content is already too high, no addition 90 of ore is made until it falls to the desired percentage or to some value slightly below this. 95

During the heat, analysis of the slag at frequent intervals for iron oxide is desirable and the smaller and more frequent the individual ore additions, the closer to the desired percentage 5 the iron oxide in the slag can be held.

Continuous feeding of iron ore or of other oxidizing agent is within the scope of the invention as is the adjustment of the oxygen content, free or combined, of the furnace 10 gases, provided in both instances the purpose of such procedures is to maintain the iron oxide content of the slag at some predetermined value or values.

The novel method by which the percentage 15 of iron oxide appropriate in the slag for any given furnace and product constitutes a necessary and vital part of my new process for the manufacture of open hearth steel. This method involves the employment of a fundamental relationship which I have found to obtain 20 between rate of carbon elimination, the FeO content of the slag (total iron calculated to FeO), and the carbon content of the metal bath. If

$$25 \quad \frac{dx}{dt}$$

represents the rate of carbon elimination (in 30 per cent carbon per minute) from the metal bath at the time "t", "x" the coincident percentage of carbon in the metal bath, and "w" that of FeO in the slag, then this fundamental relationship may be expressed in the form of the following equation:

$$35 \quad \frac{dx}{dt} = akw \left( 1.08 w - \frac{1}{x} \right) \quad (I)$$

where  $k$  is a constant, "a" is a numerical factor derived from the equilibrium constant of 40 the reaction  $\text{FeO} + \text{C} \rightarrow \text{CO} + \text{Fe}$ , and may for practical purposes be assumed to have a value of .0000757, but is known to vary slightly with the temperature of the metal bath. This equation, when integrated between the limits 45  $x_2$  and  $x_1$ , representing initial and final carbon contents, yields the elapsed time equation:

$$50 \quad T = 12,230 \left( \frac{x_2 - x_1}{kw^2} \right) + \frac{26,080}{kw^3} \log \left( \frac{1.08wx_2 - 1}{1.08wx_1 - 1} \right) \quad (II)$$

where  $T$  is the time in minutes required for the carbon content of the metal bath to fall 55 from  $x_2$  percent to  $x_1$  percent while the FeO content of the slag is maintained at  $w$  percent.

Equations (I) and (II) I have found to hold to a degree of approximation entirely 60 sufficient for practical purposes during the finishing period of the heat, after the metal is melted and covered with a continuous layer of slag of workable viscosity.

The constant  $k$  which occurs in the two 65 equations is a constant only in the sense of be-

ing a "furnace constant", i. e. it varies from furnace to furnace, even at times when the furnaces in question are ostensibly of the same design and capacity. The value of  $k$  is undoubtedly controlled not only by hearth area, depths of metal and slag layers, but also by the rate at which oxygen is transferred from the furnace gases to the slag layer, where the reaction  $4\text{FeO} + \text{O}_2 = 2\text{Fe}_2\text{O}_3$  is constantly occurring. The oxygen in question may be free oxygen,  $\text{CO}_2$ , or  $\text{H}_2\text{O}$  in the furnace gases. The  $\text{Fe}_2\text{O}_3$  thus formed acts like the  $\text{Fe}_2\text{O}_3$  introduced by the iron ore additions in reducing the carbon content of a metal bath. This rate of oxygen transfer is 70 a characteristic of flame temperature and combustion conditions and is therefore included within the furnace constant  $k$ . A change of fuel, of burner design, design of ports, and checker-work all may affect the 75 value of  $k$ .

The actual value for any given set of furnace conditions can be determined by substituting observed values in Equation (I) and solving for  $k$ . The rate term

$$80 \quad \frac{dx}{dt}$$

can be readily obtained graphically from the carbon-time curve for any selected heat. An alternative method for arriving at  $k$  is to employ Equation (II), substituting observed values for  $x_1$ ,  $x_2$ ,  $T$ , and  $w$ . In this case, however, the method is not exact unless  $w$  remains substantially constant during the period of observation or unless the square root of the mean square of a number of values of  $w$  taken at substantially uniform small intervals is used.

In actual practice tables or curves may be 95 used, derived from Equations (I) or (II) or both, thus avoiding all unnecessary calculations while the heat is in progress.

From the equations or from such above mentioned tables or curves, it is readily possible to choose for any particular carbon content desired at the finish of the refining process, such a value of FeO in the slag as will yield a rate of elimination  $\left( \frac{dx}{dt} \right)$  at said finish-

100 ing time of from 0 to, say, 0.004% carbon per minute. The lower the rate the lower will be the iron oxide in both slag and metal and the smaller the amount of dissolved iron oxide and gases which have to be removed from the metal by deoxidizers or by effervescence (in the case of "open" steels) for the production of a clean steel. The practical value of obtaining in the furnace a metal bath containing 105 iron oxide and oxygen-containing gases in the minimum practicable quantity before adding ferromanganese, ferrosilicon, etc., will be apparent to those skilled in the art.

I have found that in the case of a number 110 of 100-ton stationary basic open-hearth fur-

naces the constant  $k$  as determined by experiment has a value which varies over some such range as 0.04 to 0.15.

I give below the calculated time (T) required to drop the carbon content from 0.50% ( $x_2$ ) to various lower values ( $x_1$ ) for two different fixed percentages of iron oxide ( $w$ ) in the slag, where the furnace constant ( $k$ ) is equal to 0.05.

|    | Per cent carbon $x_2$ | Per cent carbon $x_1$ | Time required when $w=20\%$ | Time required when $w=30\%$ |
|----|-----------------------|-----------------------|-----------------------------|-----------------------------|
|    |                       |                       | Minutes                     | Minutes                     |
| 15 | 0.50                  | 0.40                  | 68                          | 29                          |
|    | 0.50                  | 0.30                  | 138                         | 59                          |
|    | 0.50                  | 0.20                  | 213                         | 90                          |
|    | 0.50                  | 0.15                  | 266                         | 107                         |
|    | 0.50                  | 0.10                  | 289                         | 125                         |
|    | 0.50                  | 0.08                  | 330                         | 133                         |
|    | 0.50                  | 0.06                  | 368                         | 143                         |
|    | 0.50                  | 0.05                  | 411                         | 149                         |
| 20 | 0.50                  | 0.04                  | ∞                           | 158                         |
|    | 0.50                  | 0.03                  | ∞                           | ∞                           |

The times as calculated were found to agree closely with those actually occurring in practice.

This table may be written to indicate rate of carbon elimination, as follows:—

|    | Per cent carbon | FeO 20% | FeO 30% |
|----|-----------------|---------|---------|
| 30 | 0.40-0.30       | .0016   | .0035   |
|    | 0.30-.20        | .0016   | .0035   |
|    | .20-.15         | .0015   | .0035   |
|    | .15-.10         | .0014   | .0035   |
|    | .10-.08         | .0014   | .0033   |
|    | .08-.06         | .0012   | .0033   |
|    | .06-.05         | .0007   | .0029   |
| 35 | .05-.04         | 0       | 0       |

Suppose it were required to make steel containing 0.04 C. at the finish of the refining operation. Evidently from the above tables such a steel could not be made at all with a slag containing 20% FeO. The table shows that with a 30% FeO slag it would be feasible to produce a 0.04 C. steel, and that the rate of carbon elimination is relatively rapid at the time this carbon percentage is reached.

Let it be assumed that a rate of .0020 instead of .0029 is decided upon as the proper rate of carbon elimination for minimizing the non-metallic inclusions, then the value of "w" for this particular condition can be determined from Equation (I).

Obviously the requisite information as to various percentages of carbon content, rate of elimination and FeO percentage in slag can be conveniently tabulated or graphically shown in curves.

Examples of such curves are shown in the accompanying drawing and are self-explanatory.

The melter can by observation of the rate of carbon elimination (which is dependent upon the iron oxide content of the slag) as shown by the curve, ascertain with sufficient accuracy, even without analysis, the iron-

oxide content of the slag and act accordingly. Such a procedure is obviously within the scope of my invention.

In carrying out the process the melter will know in advance the desirable percentage of FeO in the slag during the refining stage, and will know that the best results can be obtained by maintaining this percentage until the desired carbon content is obtained.

Preferably the percentage of FeO in the slag is determined at the close of the melting stage, brought to the desired percentage if necessary, and maintained thereafter, but obviously it can be obtained during the refining stage and modified as may be required.

It is a common mistake in practice to add too much iron oxide ("over-oreing") so that at the time of "finishing" the heat too much iron oxide is present in the slag, and the melter has up till my invention had no means of knowing how to control the conditions. It will be understood that the heat is "finished" when the desired carbon point is reached and that further elimination of carbon by iron oxide in the slag is then stopped or slowed up by the addition of deoxidizers such as ferromanganese or ferrosilicon.

If too little oxide of iron is present toward the close of the refining stage, the elimination of carbon and the duration of the heat are unduly prolonged. When this condition is reached, it is necessary to add more iron oxide, which at the stage of the operation is undesirable in any event, and usually too much is added with the detrimental results above referred to.

By carrying out the process according to my invention, these difficulties are obviated.

It has hitherto been common practice in basic open-hearth "melting" to proceed more or less in accordance with a certain standardized program, subject, however, to considerable flexibility even in the case of a fixed charge composition. Where the initial metal charge consists, as it usually does, of scrap steel and pig iron, it is customary to charge the scrap first, on top of the limestone which has been previously laid on the bottom of the hearth, and then to charge the pig iron after the scrap has started to melt. After the pig iron, either solid or molten, is added, the "lime boil" sets in vigorously and continues as a rule for 2 to 4 hrs. This "boil" is due to evolution of carbon dioxide from the limestone ( $CaCO_3$ ) in the charge.

Due to increasing hydrostatic pressure of the metal and thermal dissociation of  $CaCO_3$ , lime is disengaged from the bottom and rises to the top of the slag where it continues to go into solution in the slag. By the time the metal charge has melted down, the "lime boil" has as a rule come to an end, although boiling in isolated spots may continue for a longer interval of time. Solution of the calcined limestone, or  $CaO$ , which rises to the slag

surface and floats thereon, may not be complete until the lapse of several hours following the melting of the metal charge. The slag is not entirely "shaped up" until the floating lime lumps have dissolved in the slag, although toward the end of lime solution the few scattered lumps which remain have only a very small effect on the "shaping up" of the slag.

When the metal charge is melted, a spoon or small hand ladle is introduced beneath the slag and a test sample of metal removed from the bath. This is poured into a small cast-iron mold and allowed to solidify. It is removed from the mold while at a red or yellow heat and cooled in water more or less slowly, but at a more or less fixed rate. The test piece is then broken and the carbon content estimated from the appearance of the fracture. The test piece may, if desired, be sent to the chemical laboratory for a rapid carbon analysis for check purposes. The carbon content of the metal at melting down is important, since it is used by the melter in deciding how heavy an initial addition of iron oxide (usually as iron ore) is proper under the circumstances. In case the heat melts at a relatively low carbon content, "oreing" may be dispensed with entirely and, in extreme cases, recourse may be had to a re-carburizing addition of pig iron or spiegel. It is however, generally agreed that good practice requires a carbon content at melting sufficiently high to require a certain amount of "oreing".

It is at the conclusion of this melting stage that the so-called refining or finishing stage of the heat begins.

According to my invention, it is at this time that the iron oxide (FeO) content of the slag is determined by chemical analysis, and successive analyses are made from time to time, during the refining stage, and the iron oxide content of the slag accordingly so adjusted as to keep it substantially of a constant percentage, as decided upon and determined by the methods above described. It is desirable to make carbon determinations coincident with the iron oxide analyses. While it is desirable to correctly adjust the slag composition at the beginning of the refining stage, obviously this may be effected later, as long as sufficient time is permitted for the reactions, above described, between the metal and the slag, to take place at the desired rate of carbon elimination.

It is to be understood that the refining of the steel is otherwise carried out in the usual way including the maintenance of the proper fluidity of the slag, and the addition, at the proper time, of deoxidizers such as ferromanganese or ferrosilicon, so that the metal bath may be cleansed of dissolved and suspended oxides before it is tapped from the furnace.

The result of the application of my inven-

tion is that the melter, instead of carrying out the refining by more or less haphazard methods based largely on his skill and experience, is furnished with an additional guiding factor of control whereby better final results may be obtained.

I claim:

1. The process of making open-hearth steel which comprises melting the charge and thereafter refining the steel in the presence of a slag in which there is maintained a substantially constant percentage of iron oxide, the said constant percentage of iron oxide being maintained by determining the iron oxide content of the slag from time to time in the course of the refining, and adjusting such content if necessary to bring it to the constant percentage.

2. The process of making open-hearth steel which comprises melting the charge, and refining the steel after the melting in the presence of a slag having a substantially constant percentage of iron oxide determined according to the equation

$$\frac{dx}{dt} = .0000757 kw \left( 1.08 - \frac{1}{x} \right)$$

in which

$$\frac{dx}{dt}$$

is the desired rate of carbon elimination,  $k$  is a constant,  $w$  is the percentage of FeO in the slag and  $x$  the coincident percentage of carbon in the bath at time  $t$ , the said constant percentage of iron oxide being maintained by determining the iron oxide content of the slag from time to time in the course of the refining, and adjusting such content, if necessary, to bring it to the said constant percentage.

In testimony whereof, I affix my signature.

ALEXANDER L. FEILD.

90.

95.

100.

105.

110.

115.

120.

125.

70.

75.

80.

85.

105.

115.

125.